

J. H. PAYNE.  
PROCESS OF AGGLOMERATING FINE ORES.  
APPLICATION FILED FEB. 21, 1914.

1,114,029.

Patented Oct. 20, 1914.



# UNITED STATES PATENT OFFICE.

JAMES H. PAYNE, OF BALTIMORE, MARYLAND.

## PROCESS OF AGGLOMERATING FINE ORES.

1,114,029.

Specification of Letters Patent.

Patented Oct. 20, 1914.

Application filed February 21, 1914. Serial No. 820,156.

*To all whom it may concern:*

Be it known that I, JAMES H. PAYNE, a citizen of the United States, residing at Baltimore, in the State of Maryland, have invented or discovered certain new and useful Improvements in Processes of Agglomerating Fine Ores, of which the following is a specification, reference being had therein to the accompanying drawings.

This invention relates to the nodulizing of fine ores, containing considerable quantities of sulfur, which cannot be conveniently nodulized in accordance with the processes described in most of the prior patents on nodulizing, for the reason that the combustion of the large quantities of sulfur present generates a sufficient amount of heat to carry the temperature of the ore under treatment to a point somewhat above that necessary for the incipient fusion which produces the nodulizing.

In the well known ore nodulizing process, which consists in heating ore to the point of incipient fusion while it travels downwardly through an inclined rotating cylinder, care must be taken that the temperature of the ore does not appreciably exceed the point of incipient fusion because if this condition occurs the ore soon sticks to the wall of the furnace in such a hard crust as to soon choke the kiln, and further because when the ore becomes heated to too soft a state large unmanageable fused masses are produced which stop the operation of the process. In the nodulizing of certain classes of ore, particularly copper ores containing considerable quantities of metal sulfids, which ores are commonly referred to as "copper bearing pyrites", and "copper bearing pyrrhotite", the sulfur of the ore in burning is liable to produce this excessively high temperature above referred to, and it is one of the objects of the present invention to prevent the formation of this excessively high temperature by presenting any material amount of combustion of the sulfur of the ore. I have found that a convenient way of preventing the combustion of the sulfur, is by preventing the entrance of the air necessary for such combustion, thereby maintaining a substantially non-oxidizing condition, which may or may not be actually reducing, within the rotating furnace, in which the process is being carried out. The admission of air in carrying out the present invention, is restricted substantially to that which is neces-

sary for the combustion of the fuel injected at the lower end of the furnace.

In carrying out my process the apparatus shown by way of example in the annexed drawings may be employed.

In said drawings Figure 1 represents a vertical section of a furnace suitable for use in the process, with the necessary attachments thereto, and Fig. 2 represents a cross section of the apparatus shown in Fig. 1, said section being taken on the line 2—2 of Fig. 1, looking in the direction of the arrow.

In carrying out the process in the apparatus shown, the ore may be introduced by means of a spout 4, at the upper end of a rotating furnace 5, which is interiorly provided with a lining of refractory fire-brick or the like 6, and which furnace may be caused to rotate by means of the gears 7 and 8, in the usual manner.

At the lower end of the furnace 5, I provide a hood 9, which fits closely against the end of the rotating furnace 5, suitable sand seals or the like being provided if necessary or desired, in order to exclude the entrance of material quantities of air around the edges of the hood, or between the hood and the furnace 5. At 10 is shown a fuel inlet, and at 11 is shown an air inlet for producing a substantially non-oxidizing flame, for heating the ore to the nodulizing temperature, the fuel and air inlet being provided with suitable valves 15 and 16, respectively, for regulation.

The ore in gradually advancing from the spout 4 to the outlet end of the furnace, becomes gradually heated to the temperature necessary for nodulization, while the exclusion of air prevents the combustion of the liberated sulfur, thereby preventing the over-heating which would cause partial liquefaction of the ore under treatment, that is, would prevent the nodulization and would cause the molten or semi-molten ore to adhere to the walls of the furnace, which would either choke up the furnace or would form large unmanageable masses, fused together, which would not readily discharge from the lower end of the furnace, and thereby render the same inoperative. At 12 is shown an outlet for the nodulized ore, which may be provided with a suitable valve 13, which remains closed by gravity except when ore is coming out, and the outlet 12 discharges into a car or the like 14, for carrying the nodulized ore to a suitable blast

furnace or other device in which it is to be used.

In order to permit ready access to the interior of the rotating kiln for periodically cleaning or repairing or the like, the hood 9 is preferably mounted on small trucks so that it can be moved back when desired.

It will be noted that while the flap valve 13 will be open during the discharge 10 of the material from the spout 12, the spout 12 itself at that time will be full of ore being discharged so that no material amounts of air can enter at this point.

A considerable quantity of the sulfur of 15 the ore may distil therefrom in the form of elemental sulfur, which may or may not be in sufficient quantities to recover in merchantable form, but whether the sulfur is recovered or not is rather immaterial in the 20 present process, which relates to the nodulization of ore, and not to the production of sulfur as its principal feature. Moreover the prevention of the combustion of the sulfur likewise prevents the formation of large 25 quantities of sulfur dioxide which being discharged into the atmosphere would cause a material nuisance to plant life in the vicinity of the works.

A second difficulty is often met with in 30 the treatment of sulfid ores of the class herein referred to, namely that the temperature of material even when heated so as to avoid oxidization as above referred to, has only a very short range between the point of incipient fusion and the point of more or less 35 complete fusion, and in certain cases, I accordingly add a fusion retarding agent to the ore, as in my copending application No. 760,260, filed April 10, 1913. As in said 40 prior application above referred to, I may add a suitable material to prevent over-fusion of the mass of material, that is to say with ores of an acid nature I may add silica or sand, while with ores of an alkaline nature I may add lime or the like, or in either 45 case I may add a substance of which the decomposition is endothermic, such as calcium sulfate or the like, and it is of course understood, that in place of pure silica, pure lime, or pure calcium sulfate, I may employ ores 50 containing copper or other valuable metal, in which is also contained the silica, lime, or calcium sulfate, or other material to be employed for the purpose of preventing over-fusion.

While the step of preventing oxidation of the sulfur is in many cases sufficient to effect good nodulization of the sulfid ores, I find that in certain cases it is advisable to 55 combine this step with the addition of a retarding agent as above stated.

It is obvious that various fuels may be used, such as gas, oil, or powdered coal, provided the precaution is taken to burn 60 them without a material excess of air in

order that the heated gases resulting may be practically free from oxidizing effect upon the sulfur of the ore.

Various modifications of other portions of the process may be made without departing 70 from the spirit of my invention.

Having thus described my invention what I claim is:

1. A process of nodulizing ores containing sulfur in material amounts which comprises 75 heating said ore to a point of incipient fusion while agitating the same, and while avoiding the presence of sufficient free oxygen to burn the sulfur of said ore, thereby avoiding over-fusion of the ore. 80

2. A process of treating ores containing material quantities of sulfur, which comprises heating a stream of said ore, while agitating and rolling the particles thereof; introducing a flame of air and fuel in 85 counter current with said stream of ore, while preventing the entrance of sufficient air, over the amount necessary for the combustion of the fuel, to burn material quantities of the sulfur, and discharging the 90 treated ore at the lower end of the furnace.

3. A process of agglomerating fine ores containing material quantities of sulfur, which comprises heating a continuous stream of said ore while agitating and rolling the 95 particles thereof, introducing a flame of air and fuel in counter current to said stream of ore, while preventing the entrance of sufficient air, over the amount necessary for the combustion of the fuel, to burn material quantities of the sulfur, heating said 100 ore by means of said flame to the point of incipient fusion, and discharging the resulting nodules at the lower end of the furnace.

4. A process of agglomerating fine ores 105 containing material quantities of sulfur, which comprises nodulizing said ore while agitating and rolling the ore particles by applying heat practically devoid of oxidizing action upon the sulfur contained in the ore. 110

5. A process of nodulizing ore containing sulfur in the form of metal sulfid, which comprises heating said ore, by a flame applied thereto, to a temperature sufficient for incipient fusion, agitating said ore during 115 said heating operation, and avoiding contact of said ore with sufficient amounts of free oxygen to burn the sulfur.

6. A process of nodulizing sulfid ores, which comprises mixing therewith a substance capable of preventing over-fusion, heating said mixture to a nodulizing temperature, while avoiding the presence of free oxygen in amounts sufficient to burn material quantities of the sulfur content of 120 said ore.

7. A process of nodulizing sulfid ores, which comprises mixing therewith a calcareous material for the purpose of preventing over-fusion, heating said mixture to a 125 130

nodulizing temperature, while avoiding the presence of free oxygen in amounts sufficient to burn material quantities of the sulfur content of said ore, and while rolling and

5 agitating the ore particles.

8. A process of nodulizing sulfid ores, which comprises mixing therewith a substance of which the decomposition is endothermic, heating said mixture to a nodulizing

10 ing temperature, while avoiding the presence of free oxygen in amounts sufficient to burn material quantities of the sulfur content of said ore, and while rolling and agitating the ore particles.

9. A process of nodulizing sulfid ores, 15 which comprises mixing therewith calcium sulfate, heating said mixture to a nodulizing temperature, while avoiding the presence of free oxygen in amounts sufficient to burn material quantities of the sulfur content of 20 said ore, and while rolling and agitating the ore particles.

In testimony whereof I affix my signature, in presence of two witnesses.

JAMES H. PAYNE.

Witnesses:

L. R. O'HARA,  
Wm. S. TAYLOR, Jr.